

# UNITED STATES PATENT OFFICE.

CHARLES BASKERVILLE, OF NEW YORK, N. Y., ASSIGNOR TO WELSBACH LIGHT COMPANY,  
OF GLOUCESTER, NEW JERSEY, A CORPORATION OF NEW JERSEY.

## METHOD OF MAKING A SOLUTION OF RARE-EARTH METALS.

No. 873,205:

Specification of Letters Patent.

Patented Dec. 10, 1907.

Application filed June 15, 1905.—Serial No. 265,440.

*To all whom it may concern.*

Be it known that I, CHARLES BASKERVILLE, a citizen of the United States, residing at New York, in the county of New York and State of New York, have invented certain new and useful Improvements in Method of Making a Solution of Rare-Earth Metals, of which the following is a specification.

My invention relates to improvements in methods for the obtaining in solution or recovery of the oxids of cerium, thorium, zirconium, the ordinarily insoluble rare earths, as well as many of the rare earth minerals, as monazite sand and the like.

The object of my invention has for its purpose quickly and cheaply obtaining in solution the oxids of the above named elements and those of the rare earths and like substances, and also a recovery of the same from broken down Welsbach mantles in such a form as to be easily applied and used again in connection with newly woven filaments.

The invention consists of well defined steps and certain procedure which will be hereinafter more clearly described and particularly pointed out in the appended claims.

It is known that the oxids of thorium, zirconium, the rare earth oxids and minerals as monazite sands together with cerium dioxid do not dissolve completely either in strong or dilute hydrochloric acid when heated under ordinary atmospheric pressure, but I have found by experiment that the above mentioned substances will dissolve readily when heated with concentrated hydrochloric acid under pressure in a closed vessel.

In the use of sulfuric acid, the sulfates formed are only slightly soluble in water and must be dissolved in very cold water or an insoluble basic sulfate will be produced, or after solution a slight rise of temperature will produce certain crystalline compounds which go back into solution only with great difficulty.

The chlorids of these metals, cerium, thorium, zirconium and rare earths, are all quite soluble in water, and can be had and used in the concentrated form if so desired and not in dilution, the condition one must work with in sulfates. The cerium oxid goes into solution with sulfuric acid only with exceeding slowness, often not at all, and usually requires fusion with alkalies or alkaline sulfates. For the above reason, I have found that the use of hydrochloric acid is advantageous and

preferable in forming a compound which is quite soluble in water and may be had in a very concentrated form. I have discovered in dissolving the above stated substances in acids under pressure the activity of the acids is greatly increased and the substances are readily dissolved.

In recovering the oxids of the rare earths in useless and broken Welsbach mantles, the remnants of the mantles may be acted upon with nitric acid under similar conditions of pressure.

The method of operation of my invention is as follows: I take the substances containing the ordinarily insoluble oxids of cerium, thorium, zirconium, rare earth oxids or monazite sands and finely sub-divide the same in any suitable manner. This powder is placed in preferably glass tubes with an excess of hydrochloric acid. The tubes are sealed and then heated for variable lengths of time at a temperature of from 140° to 200° centigrade. The pressure developed in the sealed tubes increases the activity of the acid and the oxids above mentioned are readily obtained in solution.

It will also be understood that instead of creating the pressure within the tube or other vessel by sealing the same and applying heat, which I have found the most efficient and the preferred manner of carrying out my invention, I do not wish to limit myself to this specific arrangement, as other means and material may be adopted, as for example, a pressure pump connected to the heating vessel, which will effect the same function of sustaining an atmosphere in the tube or other vessel under pressure. If so desired, metal, earthenware or other vessels may be used, and other acids may also be employed instead of hydrochloric acid.

Having now fully described my invention, what I claim as new and desire to secure by Letters Patent is as follows:

1. The method of preparing a solution containing a rare earth metal, which comprises heating a compound of said metal with a mineral acid and under high pressure.

2. The method of preparing a solution containing a rare earth metal which comprises heating a compound of said metal in a finely divided state with hydrochloric acid and under high pressure.

3. The method of preparing a solution containing a rare earth metal which com-

prises first, finely sub-dividing the substance containing the metal, second, heating the same under high pressure and in an excess of hydrochloric acid.

5 4. The method of preparing a solution containing a rare earth metal which comprises first, finely sub-dividing the substance containing the metal, second, heating the same to a temperature from 140° to 200° C 10 under high pressure and in an excess of hydrochloric acid.

5. The method of preparing a solution containing the rare earth metals of Welsbach mantle remnants, which comprises heating 15 the remnants under high pressure in an excess of mineral acid.

6. The method of preparing a solution containing the rare earth metals of Welsbach mantle remnants, which comprises heating 20 the remnants under high pressure in an excess of mineral acid, evaporating the excess of acid and diluting the residue.

7. The method of preparing a solution containing a rare earth metal which comprises heating a compound of said metal under pressure in an aqueous solution of a mineral acid, said pressure being created by heating the solution of the acid.

8. The method of preparing a solution 30 containing a rare earth metal which comprises heating a compound of said metal in a finely divided state under pressure in an

aqueous solution of a mineral acid, said pressure being created by heating the solution of the acid.

35

9. The method of preparing a solution containing a rare earth metal which comprises first finely sub-dividing the substance containing the metal, second, heating the same under high pressure in an aqueous solution of an excess of a mineral acid, said pressure being created by heating the solution of the acid.

40

10. The method of preparing a solution containing a rare earth metal which comprises first, finely sub-dividing the substance containing the metal, second, heating the same under pressure and a temperature from 140° to 200° C. in an aqueous solution of a mineral acid, said pressure being created by 45 heating the solution of the acid.

11. The method of preparing a solution containing the rare earth metals of Welsbach mantle remnants which comprises heating the remnants under high pressure in an 50 aqueous solution of an excess of acid, said pressure being created by heating the solution of the acid.

55

In testimony whereof I affix my signature in presence of two witnesses.

CHARLES BASKERVILLE.

Witnesses:

HERBERT F. SILL,  
N. R. GRAHAM.